

April 14, 1970

HIROMU UCHIDA ET AL

3,506,413

SURFACE TREATED STEEL SHEET SUITABLE FOR FORMING

Filed Oct. 2, 1967

3 Sheets-Sheet 1

FIG. 1



INVENTORS

HIROMU UCHIDA  
TOSHIO HERAI  
YASAYUKI TANIGUCHI  
HIDESHI SATO

BY *Mark G. and Toren*  
*Attorneys*

April 14, 1970

HIROMU UCHIDA ET AL

3,506,413

SURFACE TREATED STEEL SHEET SUITABLE FOR FORMING

Filed Oct. 2, 1967

3 Sheets-Sheet 2

FIG. 2



FIG. 3



April 14, 1970

HIROMU UCHIDA ET AL

3,506,413

SURFACE TREATED STEEL SHEET SUITABLE FOR FORMING

Filed Oct. 2, 1967

3 Sheets-Sheet 3

FIG. 4



FIG. 5



## 1

3,506,413

SURFACE TREATED STEEL SHEET  
SUITABLE FOR FORMINGHiromu Uchida, Toshio Herai, Yasuyuki Taniguchi, and  
Hideshi Sato, Himeji-shi, Japan, assignors to Fuji Iron  
& Steel Co., Ltd., Tokyo, Japan

Filed Oct. 2, 1967, Ser. No. 704,496

Claims priority, application Japan, Sept. 30, 1966,  
41/64,574; Oct. 26, 1966, 41/70,511; Aug. 18,  
1967, 42/52,997

Int. Cl. B32b 15/04; B21c 23/32

U.S. Cl. 29—195

7 Claims

## ABSTRACT OF THE DISCLOSURE

Surface treated steel sheet suitable for forming which comprises a steel sheet having a metallic coating of zinc, lead, a zinc base alloy or a lead base alloy thereon, and a layer of a higher carboxylic acid or a higher carboxylic acid containing an amine coated on to said metallic coating. The coatings provide lubricity for forming operations, act as rust inhibitors and have advantageous properties as compared to oils or metallic soap based lubricants previously used on steel sheets in forming operations.

The present invention relates to a surface treated steel sheet suitable for forming. The surface treated steel sheet of this invention is obtained by coating a steel sheet with zinc, lead, zinc based alloy or lead based alloy (hereinafter called zinc or lead), and applying on the coated surface a layer of matter, solid at room temperatures, which comprises a higher carboxylic acid or a mixture thereof with a suitable amount of amine.

Lubricants are generally required when a steel sheet is subjected to a forming operation such as press forming. For this purpose oily products have been used. Recently attempts have been made to use metallic soap based lubricants as substitutes for the oil lubricants. The metallic soap based lubricants have excellent lubricating ability as compared with the oil lubricants. Also, the steel sheet which is coated with such soap bases is easy to handle, since the coating layer is solid and not sticky and thus it can be advantageously used as a coating material for a pre-lubricated steel sheet. On the other hand, the metallic soap based lubricants have disadvantages. A lengthy, high temperature heating period is required to dry such soap based lubricants because they are applied on the steel sheet in the form of an aqueous solution. This leads to decreased productivity and accelerates ageing of the steel sheet substrate thus deteriorating the quality and forming properties of the steel sheet.

The present inventors conducted various extensive experiments and studies in efforts to overcome the above difficulties with the metallic soap based lubricants. It has now been found that a surface treated steel sheet obtained by applying a metallic coating of zinc or lead, on a steel sheet surface and then applying on the metallic coating a layer consisting of a higher carboxylic acid or a mixture thereof with a suitable amount of amine, wherein said acid or mixture with amine is solid at room temperatures, gives as good a lubricity as that obtained by using the metallic soap based lubricants, and effectuates higher productivity without deteriorating the material quality of the steel sheet, and thus provides a very suitable form of prelubricated steel sheet.

These effects can be attributed to a number of reasons. The metallic surface of zinc, or lead present on the steel surface has a strong affinity with the higher carboxylic acid or its mixture with a suitable amount of amine (hereinafter called higher carboxylic acid based coating material). A thin layer of metallic-soap-like substance is formed

## 2

by reaction of the metallic coating with the higher carboxylic acid based coating material at the interface therebetween. The metallic-soap-like substance having a higher carboxylic acid radical is regularly oriented in respect to the steel sheet substrate and strongly bonded with the layer on the steel sheet substrate according to its formation history, thus giving a remarkable lubricating effect.

The experimental results obtained in support of the above conclusion are shown in FIG. 1. FIG. 1 shows the results of measurement of kinetic friction coefficient in a bath of stearic acid obtained with Soda's type II pendulum style tester, between a non-plated steel ball and three kinds of pins (1), (2) and (3). Pin 1 is a non-plated steel pin. Pin 2 is a steel pin which is coated with 10 g./m.<sup>2</sup> of zinc by electroplating and pin 3 is a steel pin which is coated with 100 g./m.<sup>2</sup> of lead-tin alloy (Sn: 20 wt. percent) by hot dipping. In the case of measurements below the melting point of the stearic acid, molten stearic acid was coated on the pin by hot dipping. This coated pin was used and the measurements taken in a water bath. The stearic acid used in the test contained a small amount of palmitic acid and had a melting point of 57°C. The zinc stearate corresponding to this stearic acid has a melting point of above 100°C. A metallic soap composed mainly of lead stearate also shows a melting point above 100°C. It should be noted from FIG. 1 that in both the zinc plated pin and the lead-zinc alloy plated pin, the kinetic friction coefficient tends to lower even above the melting point of the stearic acid and shows the minimum point at a temperature above 100°C. This is attributed to the fact that the formation reaction of zinc base or lead base metallic soap proceeds as the temperature increases so that the thus formed zinc stearate or lead stearate in the solid state gives boundary lubricating effects even beyond the melting point of the stearic acid.

On the other hand, in the case of the non-plated steel pin, the minimum point of kinetic friction coefficient appears at the melting point of stearic acid, and the friction coefficient increases as the temperature increases beyond the melting point. From this it can be seen that the formation of iron based metallic soap does not easily progress even with increases in temperature. Further, the kinetic friction coefficient near room temperatures shows a lower value in case of the zinc plated pin or the lead-tin alloy plated pin.

The above results indicate that when stearic acid is coated on zinc plated or lead plated steel sheet, a thin layer of substance analogous to zinc stearate metallic soap or lead stearate metallic soap is also formed at the interface between the stearic acid layer and the metallic layer of zinc or lead.

Thus it can be concluded that the excellent lubricity of the present steel sheet is based on the presence of a thin layer of metallic-soap-like substance formed on the interface between the metallic coating of zinc or lead and the higher carboxylic acid based coating material. It should be noted that the excellent lubricity can be maintained under most severe forming conditions, such as those encountered in press forming works. This maintenance of excellent lubricity under severe forming conditions is considered to be based on the fact that in the present steel sheet, both the metallic coating and the higher carboxylic acid coating react only partially, and for the most part remain unreacted on the steel sheet surface. Then, when the sheet is subjected to a press forming, the unreacted metallic coating and higher carboxylic acid react with each other to form an additional metallic-soap-like substance even when the aforesaid layer of metallic-soap-like substance is damaged by contact with the press forming tool and is thinned due to the dimensional increase of the steel sheet.

However, the above effects can be obtained only when the layer of higher carboxylic acid based coating is in the solid form at the ordinary temperatures. In case of a similar layer which is in the liquid form at the ordinary temperatures, the coating layer at portions on which heavy load is put during a severe forming work, namely at portions which require lubricant most, is squeezed out thus causing shortness of lubricant and a desirable maintenance of excellent lubricity as above cannot be obtained. For this reason, the layer of higher carboxylic acid based coating is limited to a solid form in the present invention.

The objects and advantages of the present invention will be fully understood through the following more detailed description of the present invention referring to the attached drawings, in which:

FIG. 1 is a graph showing the relation between temperatures and kinetic friction coefficient of a non-plated steel pin, an electrolytic zinc plated steel pin and a hot-dip lead-tin alloy (tin: 20 wt. percent) plated steel pin respectively with a non-plated steel ball in stearic acid; and FIGS. 2-5 are graphs respectively showing results of Fukui's Conical Cup Test and Erickson Test in the examples of the present invention.

The inventive construction of the present steel sheet 25 will be described in more detail.

As the metallic coatings applied on the steel sheet, zinc coating, lead coating or alloy coatings composed mainly of zinc or lead applied by an ordinary electrolytic platings or by an ordinary hot-dip plating are useful. Further the metal coatings applied by the above method may be subjected to thermal treatment to allow the coating metal to diffuse into the steel sheet substrate and convert the surface of the steel sheet substrate to an alloy system containing iron. This also gives effective metal coatings.

Furthermore, a thin layer of hydrated metal oxide, such as hydrated chromium oxide and/or silicon oxide, may be applied on the above metal coatings by a chemical treatment and the like for the purpose of improving paint adherence or preventing rust formation with almost no deteriorating effects on the forming quality of the present steel sheet.

The coating material, which is solid at room temperatures, for application on the steel sheet according to the present invention, is prepared by selecting higher carboxylic acids and adjusting the amount of amine to be added to the higher carboxylic acids as described herein-after.

The term higher carboxylic acid used in the present invention means any carboxylic acid having eight or more carbon atoms, which includes, for example, saturated fatty acids having no fewer carbon atoms than that in caprylic acid; corresponding unsaturated fatty acids; hydroxy carboxylic acids; naphthenic acids; dicarboxylic acids; and natural products composed mainly of the above acids, such as animal oil fatty acids, hardened animal oil fatty acids, vegetable oil fatty acids, hardened vegetable oil fatty acids, petroleum acids etc. Among these, the following are representative acids which are solid at room temperatures: caprylic acid, lauric acid, myristic acid, palmitic acid, stearic acid, arachidic acid, behenic acid, lignoceric acid, cerotic acid, montanic acid, melissic acid, elaidic acid, erucic acid, 12-hydroxy stearic acid, suberic acid, sebatic acid, hexadecane-dicarboxylic acid, naphthenic acid, tallow fatty acid, hardened fish oil fatty acid, hardened castor oil fatty acid, petroleum acid, etc.

As amines to be added to the above higher carboxylic acids, there are, for example, primary mono-amines such as lauryl amine and cyclohexyl amine; secondary mono-amines such as di-iso-propyl amine and di-cyclohexyl amine; tertiary monoamines such as triethyl amine; poly-amines such as di-amino-propane; and oxazines and imidazoles.

These amines are added to the higher carboxylic acids which are solid at room temperatures as mentioned be-

fore. However, most of these amines are liquid at room temperatures, and if these amines are added in an excessive amount, the resulting coating material will not be solid at room temperatures. Therefore it is necessary to limit the amount of amine to such amount as to maintain the coating material in the solid state at room temperatures. In most cases this requirement is satisfied by adding the amine in an amount not greater than its chemical equivalent weight to the higher carboxylic acid.

As for the method for applying the above higher carboxylic acid based coating material on the steel sheet coated with zinc or lead, the material may be heated or dissolved in an organic solvent to liquidize it and then applied on the sheet surface by roll coating, spray coating, brush coating, mop coating, dip coating, flow coating, etc. Alternatively, the solid material may be directly spread on the steel surface and then reflowed by heating with an infra-red beam, hot air, etc.

Although the primary purpose of the metallic coating is that of a reaction medium for forming the metallic-soap-like substance, it also acts as a rust preventing coating. Further, it produces uniform coatings by its affinity to the higher carboxylic acid based coating material.

Zinc or lead metallic coatings of various thickness were applied on steel sheet substrates and the higher carboxylic acid diluted in a solvent was applied thereon. The results showed that in case of the non-alloyed zinc or lead coatings, a uniform coating of the higher carboxylic acid based coating material is obtained when the zinc or lead coating is not less than 250 mg./m.<sup>2</sup>. When zinc or lead alloy coatings were used, a uniform coating of the coating material was obtained when the total content of lead or zinc in the alloy was not less than 250 mg./m.<sup>2</sup>.

An excellent forming character is obtained in these ranges.

As the amount of the metal coating is increased beyond the above mentioned quantities, the higher carboxylic acid based coating material reacts more easily with the metallic coating. It has been found that the lubricating effect by the higher carboxylic acid coating will be improved until the amount of the metallic coating or the total metal content increases to 2500 mg./m.<sup>2</sup>. However, the surface lubricating effect does not decrease and remains almost constant even when the amount of the metallic coating exceeds 2500 mg./m.<sup>2</sup>. Therefore any amount of not less than 250 mg./m.<sup>2</sup> of the metallic coating may be used. As for the rust preventing effect by the metallic coating, a better result can, of course, be obtained by a thicker coating.

A very small amount of the higher carboxylic acid based coating material which is solid at room temperatures is effective. Remarkable effects can be obtained when the coating material is used in an amount greater than 10 mg./m.<sup>2</sup>. Although the lubricating effect increases as the amount of this coating material increases, the practical upper limit of the coating material is 5 g./m.<sup>2</sup> in view of possible adherence and accumulation of the coating material on the sheet feeder or forming tools, and re-adherence of the accumulated coating material on the steel sheet, time required for removing the coating material at the last stage, and the necessity to minimize the contamination of the removing liquid.

It has been found that the following effects are obtained by adding an amine to the higher carboxylic acid, as compared to the higher carboxylic acid without addition of amine.

(1) Solubility in an organic solution is increased, and viscosity of the heated molten coating material is easily controlled in the coating operation.

(2) Affinity with the steel sheet substrate of the coating material is increased and the rust preventing effect is increased.

(3) Washing removability of the coating material by an alkaline base degreaser or an organic solvent is im-

proved. However, an amine having excessive carbon atoms and low affinity to water, such as myristyl amine, is not desirable for this particular purpose due to its low solubility in an alkaline degreaser.

Naturally, the present invention includes not only a steel sheet both sides of which are surface treated but also a steel sheet wherein only one side is surface treated and further a steel sheet wherein only a part thereof is surface treated. The latter sheets are at times suitable to certain types of forming operations.

The present steel sheets are produced in three steps; production of steel sheet substrate (non-plated), coating of metal; and application of the higher carboxylic acid based coating material. However, it is not necessary to conduct the above three steps in the same shop. Each of the steps can be done in a separate shop. The last step of applying the higher carboxylic acid based coating material may be done on the blanking line or just before the forming operation.

Any steel sheet or any steel sheet piece thus produced falls within the scope of the present invention.

Addition of colouring matter, filler or rust preventing additive in the higher carboxylic acid based coating material in an amount insufficient to change the basic nature of the coating material does not damage the specific functions of the present steel sheet.

Various advantageous properties of the present steel sheet are set forth below.

(1) Excellent formability is obtained. This is due to the excellent lubricity of the surface, and thus application of additional lubricating oil is not necessary. For this reason, the efficiency of the forming operation is remarkably improved.

(2) Since the higher carboxylic acid base material is solid, dry and not too sticky, dust does not deposit on the surface and surface defects occur far less often during the press forming. In addition to the fact that only a small amount of the coating material is required, no irregularities, no squeeze-out of the coating material and no transfer of the coating material from surface to surface is seen even when the steel sheets are piled. Therefore it is easy to control and maintain the amount of the coating material to be applied on each side of the steel sheet.

(3) Good weldability is obtained since the coated surface is dry and the higher carboxylic acid based coating material acts as fluxing agent.

(4) The higher carboxylic acid based coating material can be easily removed by an alkaline degreaser or an organic solvent. Contamination by the coating material, particularly, of the alkaline degreaser, is negligible due to the nature of the coating material and the fact that the coating material is applied in a small amount. Also, the zinc and lead based metallic coatings may be, if necessary, removed by an acid solution, such as sulphuric acid, acetic acid, hydrochloric acid, or by a strong alkaline solution. Also, if desired, only the higher carboxylic acid based coating material can be removed after the forming work and the metallic coating can be utilized as a protective and decorative layer for the final product or as a paint coating base or a base for a chemical treatment (such as chromate treatment and phosphate treatment).

(5) In the present steel sheet, if the higher carboxylic acid based coating material is removed after a forming operation and further if the zinc base metallic coating is finally removed by acid pickling, the zinc base metallic coating dissolves acting as a sacrificing anode to the steel sheet substrate during the acid pickling. The finally exposed, naked surface of the steel sheet has very high activity just as in case of cathodic acid pickling and provides an excellent base for permanent plating. When the present steel sheet is used in such applications, a thinner zinc base coating (zinc content in the coating is 250-2500 mg./m.<sup>2</sup>) is advantageous in view of economy and its easier removal. Such a metallic coating is also useful as a pre-coating for promoting a phosphate treatment applied on the steel sheet as paint base etc. and for uniformly forming such a phosphate coating.

(6) Since coating material which does not dry easily, such as a metallic soap lubricant is avoided, a long period of heating is not necessary. This results in higher productivity and avoids deterioration of the quality of the steel sheet substrate.

#### EXAMPLE 1

Various metallic coatings and higher carboxylic acid based coating material and comparison lubricating oil as defined in Table 1 were applied on a cold rolled, remined steel sheet of 0.8 mm. thickness, and results of press formability tests are shown in Table 2. From these results it is clearly understood that the present steel sheet has an excellent formability in respect of deep drawing and stretching.

TABLE 1

| Metal     | Plating method | Metallic coating |                            | Amount, g./m. <sup>2</sup> | Higher carboxylic acid base coating material and lubricant |
|-----------|----------------|------------------|----------------------------|----------------------------|------------------------------------------------------------|
|           |                | Material         | Amount, g./m. <sup>2</sup> |                            |                                                            |
| Test No.: |                |                  |                            |                            |                                                            |
| A*        |                |                  |                            |                            |                                                            |
| B**       | An.            | Electroplating   | 10                         | (1)                        | 0.2                                                        |
| C**       |                |                  |                            | (2)                        | 0.25                                                       |
| D**       |                |                  |                            | #120 machine oil           | 3                                                          |
| E*        |                |                  |                            | Commercial press oil       | 6                                                          |
| F*        | pb.            | do               | 10                         | (1)                        | 0.2                                                        |
| G**       |                |                  |                            | (2)                        | 0.25                                                       |
| H**       |                |                  |                            | #120 machine oil           | 3                                                          |
| I*        | 90 Zn, 10 Cd   | do               | 10                         | Commercial press oil       | 6                                                          |
| J**       |                |                  | 10                         | (1)                        | 0.2                                                        |
| K*        | 55 Zn, 45 Sn   | do               | 10                         | (2)                        | 0.25                                                       |
| L**       |                |                  |                            | #120 machine oil           | 3                                                          |
| M*        | Zn             | Hot dip          | 100                        | (1)                        | 0.2                                                        |
| N**       |                |                  |                            | #120 machine oil           | 3                                                          |
| O*        | 80 pb, 20 Sn   | do               | 100                        | (1)                        | 0.2                                                        |
| P**       |                |                  |                            | (2)                        | 0.25                                                       |
| Q*        |                |                  | 100                        | #120 machine oil           | 3                                                          |
| R**       | 89 Zn, 11 Fe   | ***              | 50                         | (1)                        | 0.2                                                        |
| S**       |                |                  |                            | (2)                        | 0.25                                                       |
| T**       |                |                  |                            | #120 machine oil           | 3                                                          |
| U**       | Nonplated      |                  |                            | (1)                        | 6                                                          |
| V**       |                |                  |                            | Commercial press oil       | 6                                                          |

\*Inventive steel sheet.

\*\*Comparison steel sheet.

\*\*\*Hot dip zinc plating then thermal diffusion.

(1) Palmitic acid.

(2) A mixture of one part of palmitic acid and 0.25 part of di-cyclohexyl amine dissolved in toluene was applied and dried.

TABLE 2

| Test No.: | Conical cup test value | Erichsen value |
|-----------|------------------------|----------------|
| A*        | 37.4                   | 10.4           |
| B*        | 37.5                   | 10.6           |
| C*        | 38.5                   | 9.8            |
| D**       | 37.9                   | 10.2           |
| E*        | 37.2                   | 10.8           |
| F*        | 37.1                   | 10.8           |
| G**       | 38.0                   | 10.1           |
| H**       | 37.7                   | 10.2           |
| I*        | 37.2                   | 10.5           |
| J**       | 38.4                   | 10.0           |
| K*        | 37.4                   | 10.3           |
| L**       | 38.5                   | 9.9            |
| M*        | 37.8                   | 10.4           |
| N**       | 38.8                   | 9.7            |
| O*        | 37.3                   | 11.0           |
| P**       | 38.0                   | 10.2           |
| Q*        | 38.0                   | 10.5           |
| R**       | 38.9                   | 9.8            |
| S**       | 37.8                   | 10.3           |
| T**       | 37.7                   | 10.2           |
| U**       | 38.2                   | 10.0           |
| V**       | 37.9                   | 10.3           |

\* Inventive steel sheet.

\*\* Comparison steel sheet.

## EXAMPLE 2

1 g./m.<sup>2</sup> of zinc coating was applied on a cold rolled rimmed steel sheet of 0.8 mm. thickness, and then palmitic acid dissolved in toluene was coated on the surface and dried. The amount of the palmitic acid coating was increased stepwise and press formability of the steel sheet was tested. The results are shown in Table 3.

TABLE 3

| Amount of Palmitine acid coating (mg./m. <sup>2</sup> ) | Conical cut <sup>1</sup> value (mm.) | Maximum stretching <sup>2</sup> height (mm.) |
|---------------------------------------------------------|--------------------------------------|----------------------------------------------|
| 0                                                       | 38.8                                 | 8.9                                          |
| 2                                                       | 38.5                                 | 9.6                                          |
| 10                                                      | 37.2                                 | 13.5                                         |
| 50                                                      | 37.0                                 | 13.3                                         |
| 100                                                     | 36.5                                 | 13.7                                         |
| 200                                                     | 36.5                                 | 14.0                                         |

<sup>1</sup>By a round-bottom punch. Blank dia: 50 mm.<sup>2</sup> By a flat-bottom punch of 40 mm. dia. Frange clamped.

From the results of this example it is seen that an excellent forming quality can be obtained when the amount of palmitic acid coating is not less than 10 mg./m.<sup>2</sup>. Similar results were obtained when other coating materials were used.

## EXAMPLE 3

10 g./m.<sup>2</sup> of zinc electroplating was applied on cold rolled, rimmed steel sheets of 0.8 mm. thickness, and then the following treatments were applied. Results of various tests are shown in Table 4. Testpieces A-K are present inventive steel sheets and L-P are comparison steel sheets.

## Treatments

## Testpieces (inventive steel sheets):

- A—Lauric acid as toluen solution was applied and dried (non-volatile matter: 200 mg./m.<sup>2</sup>)  
 B—Palmitic acid as toluen solution was applied and dried (non-volatile matter: 200 mg./m.<sup>2</sup>)  
 C—Stearic acid as toluen solution was applied and dried (non-volatile matter: 200 mg./m.<sup>2</sup>)  
 D—Behenic acid as toluen solution was applied and dried (non-volatile matter: 200 mg./m.<sup>2</sup>)  
 E—Sebacic acid as toluen solution was applied and dried (non-volatile matter: 200 mg./m.<sup>2</sup>)  
 F—Beef tallow fatty acid as toluen solution was applied and dried (non-volatile matter: 200 mg./m.<sup>2</sup>)  
 G—Palm oil fatty acid as toluen solution was applied and dried (non-volatile matter: 200 mg./m.<sup>2</sup>)

- H—Hardened castor oil fatty acid as toluen solution was applied and dried (non-volatile matter: 200 mg./m.<sup>2</sup>)  
 I—Hardened fish oil fatty acid as toluen solution was applied and dried (non-volatile matter: 200 mg./m.<sup>2</sup>)  
 J—Palmitic acid was melted by heating and applied (non-volatile matter: 200 mg./m.<sup>2</sup>)  
 K—Solid palmitic acid was directly spread on the steel surface and melted by an infra-red lamp (non-volatile matter: 200 mg./m.<sup>2</sup>)  
 10 Test pieces (comparison):  
 L—Zinc electroplating was applied on one side and press oil (also for rust prevention was applied 3 g./m.<sup>2</sup>).  
 M—Only zinc electroplating on one side.  
 15 N—Same treatment as A was applied on non-plated, cold rolled, rimmed steel sheet of 0.8 mm. thickness.  
 O—Same treatment was C was applied on non-plated, cold rolled, rimmed steel sheet of 0.8 mm. thickness.  
 P—Non-plated cold rolled, rimmed steel sheet of 0.8 mm. was directly tested.

TABLE 4.—FORMABILITY  
[Inventive steel sheets]

|                           | Unical cup value | Maximum punch stretching height | Removability of treating material | Surface finish |
|---------------------------|------------------|---------------------------------|-----------------------------------|----------------|
| Test pieces:              |                  |                                 |                                   |                |
| 30 A                      | 37.0             | 13.7                            |                                   |                |
| B                         | 36.5             | 14.2                            |                                   |                |
| C                         | 36.2             | 14.6                            |                                   |                |
| D                         | 36.3             | 14.6                            |                                   |                |
| E                         | 36.9             | 13.5                            |                                   |                |
| F                         | 36.2             | 14.2                            | Good..... Dry.                    |                |
| G                         | 37.1             | 14.0                            |                                   |                |
| H                         | 37.0             | 14.5                            |                                   |                |
| I                         | 36.6             | 14.3                            |                                   |                |
| J                         | 36.5             | 14.1                            |                                   |                |
| K                         | 36.4             | 14.3                            |                                   |                |
| [Comparison steel sheets] |                  |                                 |                                   |                |
| 40 L                      | 38.9             | 9.7                             |                                   |                |
| M                         | 39.2             | 9.0                             |                                   |                |
| N                         | 38.0             | 11.8                            | Good..... Dry.                    |                |
| O                         | 38.2             | 10.2                            |                                   |                |
| P                         | 38.5             | 10.0                            |                                   |                |
|                           |                  |                                 |                                   |                |

## Formability testing

*Conical cup test.*—No lubricant was used. Same as in Example 2 except conical cup testing was made with the treated surface faced on a die side.

*Punch stretching test.*—Measured with the treated surface faced on the punch side.

*Treatment material removing test.*—Aqueous solution of parkocleaner N 958 (10 g./l.) was used. Those which show complete wettability with water of the zinc based metallic coating or the naked steel sheet surface after spray washing with an aqueous solution at 60° C. for 20 seconds are regarded as "good."

50

## EXAMPLE 4

Various zinc base metallic coatings were applied on cold rolled, rimmed steel sheets (A-J) of 0.8 mm. thickness, and a toluene solution of palmitic acid was coated on the one side of the steel sheets and dried to give 2 g./m.<sup>2</sup> of non-volatile matter coating. Forming qualities of these steel sheets and the comparison steel sheets B' and K were tested. The results are shown in Table 5.

## Steel sheets

- A—Coated with hot dip zinc coating of 100 g./m.<sup>2</sup>  
 B—Coated with hot dip zinc coating of 100 g./m.<sup>2</sup> and heat treated to alloy the zinc coating with part of the steel sheet substrate thus forming a zinc-iron alloy layer.  
 B'—Commercial press oil was applied on similar steel sheet as B  
 (Comparison)  
 C—Coated with hot dip zinc-tin alloy (Sn: 25%) plating of 100 g./m.<sup>2</sup>  
 D—Coated with zinc electroplating of 50 g./m.<sup>2</sup>  
 E—Coated with zinc electroplating of 10 g./m.<sup>2</sup>  
 F—Coated with zinc electroplating of 2 g./m.<sup>2</sup>

- G—Coated with zinc electroplating of 500 mg./m.<sup>2</sup>  
 H—Coated with zinc electroplating of 250 mg./m.<sup>2</sup>  
 I—Coated with zinc electroplating of 100 mg./m.<sup>2</sup>  
 J—Coated with zinc electroplating of 10 mg./m.<sup>2</sup>  
 K—Commercial press oil was applied on a non-plated steel sheet.  
 (Comparison)

TABLE 5

|                 | Amount of zinc coating (g./m. <sup>2</sup> ) | Conical cup value (mm.) | Maximum punch stretching height (mm.) |
|-----------------|----------------------------------------------|-------------------------|---------------------------------------|
| Steel sheets:   |                                              |                         |                                       |
| A               | 100                                          | 37.4                    | 13.3                                  |
| B               | 100                                          | 37.9                    | 12.8                                  |
| B' (comparison) | 100                                          | 38.5                    | 12.2                                  |
| C               | 75                                           | 36.1                    | 14.6                                  |
| D               | 50                                           | 37.2                    | 13.9                                  |
| E               | 10                                           | 37.0                    | 13.8                                  |
| F               | 2                                            | 36.6                    | 14.3                                  |
| G               | 500 (mg./m. <sup>2</sup> )                   | 36.5                    | 14.1                                  |
| H               | 250 (mg./m. <sup>2</sup> )                   | 37.1                    | 13.7                                  |
| I               | 100 (mg./m. <sup>2</sup> )                   | 38.4                    | 12.5                                  |
| J               | 10 (mg./m. <sup>2</sup> )                    | 38.7                    | 12.4                                  |
| K (comparison)  | 0                                            | 38.3                    | 12.1                                  |

Testing conditions are same as Example 2.

#### EXAMPLE 5

A number of test pieces similar to steel sheets A and B of Example 4 were made, and conical cup tests were done with the treated surfaces of the testpiece faced on the die side. As comparison, non-treated steel sheets A' and B' corresponding to steels A and B, were subjected to conical cup tests. Sheets A' and B' were lubricated with spindle oil on their die sides. The results are shown in FIG. 2, in which the average conical cup values of every five testpieces from the beginning of the test are plotted against the testing order.

On the other hand, the testpieces A and B were continuously subjected to Erichsen tests with the treated surface faced on the punch side, and as comparison, non-treated testpieces A' and B' corresponding to the testpieces A and B were also tested with vaseline lubricated on the punch side surface of the testpieces. Results are shown in FIG. 3, in which the ordinate shows an average value for every five testpieces.

The results indicates that the present steel sheet which are treated with palmitic acid are far more constant in their test values and do not give any effect on the tool by repetition of tests, whereas the non-treated steel sheets which are lubricated with spindle oil or vaseline only show substantial variation in their measurements, which clearly indicates the effect of burning of the metallic layer.

#### EXAMPLE 6

Testpiece A taken from a steel sheet which was coated with 10 g./m.<sup>2</sup> of zinc electroplating and subjected to chromate treatment (Cr: 30 mg./m.<sup>2</sup>) and testpiece B taken from a plated steel sheet without chromate treatment were coated with 1 g./m.<sup>2</sup> of palmitic acid as toluene solution and dried. Results of forming quality test of tests testpieces are shown in Table 6.

TABLE 6

| Testpiece: | Conical cup value (mm.) | Maximum punch stretching height (mm.) |
|------------|-------------------------|---------------------------------------|
| A          | 37.4                    | 12.1                                  |
| B          | 37.2                    | 12.5                                  |

As seen from the above results, the chromate treatment does not hinder the lubricity of the present steel sheet.

#### EXAMPLE 7

Cold rolled, rimmed steel sheets of 0.8 mm. thickness were deep drawn into a square (100 x 100 mm.) box using a square blank (220 x 220 mm.) under a blank holder pressure of about 10 tons. Steel sheets lubricated with machine oil or relatively low viscosity press oil were broken at a depth of 10 to 30 mm., while steel sheets applied with high viscosity press oil containing extreme-pressure additives and the present steel sheets which had been coated with 2 g./m.<sup>2</sup> of zinc electroplating and applied with palmitic acid as toluene solution and dried to give about 300 mg./m.<sup>2</sup> of non-volatile matter could be easily drawn without using other lubricant.

The maximum punch load in case of the present steel sheets was 5–20% lower that of the steel sheets which were applied with other oil lubricant.

#### EXAMPLE 8

Lead electroplated (plating thickness: 1 g./m.<sup>2</sup>) steel sheets of 0.8 mm. thickness were coated with various amounts of palmitic acid as toluene solution on the side and subjected to formability tests, the results of which are shown in Table 7.

TABLE 7

| Amount of palmitic acid (mg./m. <sup>2</sup> ) | Conical cup value <sup>1</sup> (mm.) | Erichsen value <sup>2</sup> (mm.) |
|------------------------------------------------|--------------------------------------|-----------------------------------|
| 0                                              | 37.8                                 | 10.5                              |
| 2                                              | 37.7                                 | 10.5                              |
| 10                                             | 37.4                                 | 11.2                              |
| 50                                             | 36.9                                 | 11.9                              |
| 100                                            | 36.6                                 | 11.7                              |
| 200                                            | 36.7                                 | 12.0                              |

<sup>1</sup> With the treated surface faced on the die side.

<sup>2</sup> The treated surface faced on the punch side.

From the above results it has been found that an excellent forming quality can be obtained when the amount of palmitic acid to be coated is not less than 10 mg./m.<sup>2</sup>.

Similar results were obtained by using other treating materials of the present invention.

#### EXAMPLE 9

The following steel sheets A to J were subjected to various tests, the results of which are shown in Table 8. Steel sheets A to E are lead-tin alloy (Sn: 15 wt. percent) hot dip plated (plating thickness, 100 g./m.<sup>2</sup>) and are treated as under on one side, and there sheets fall within the scope of the present invention. Steel sheets F to J are set forth as comparison and include plated steel sheets with various treatments and non-plated steel sheets with various treatments.

Steel sheet:

- A—Coated with lauric acid as toluene solution and dried (non-volatile matter: 200 mg./m.<sup>2</sup>)  
 B—Coated with palmitic acid as toluene solution and dried (non-volatile matter: 200 mg./m.<sup>2</sup>)  
 C—Coated with stearic acid as toluene solution and dried (non-volatile matter: 200 mg./m.<sup>2</sup>)  
 D—Coated with molten palmitic acid (non-volatile matter: 200 mg./m.<sup>2</sup>)  
 E—Spread with solid palmitic acid, which was reflowed with an infra-red lamp (non-volatile matter: 200 mg./m.<sup>2</sup>)  
 F (comparison)—Coated with rust preventing and lubricating oil in an amount of 3 g./m.<sup>2</sup>  
 G (comparison)—Non-treated, plated steel sheet  
 H (comparison)—Naked steel sheet with same treatment as A  
 I (comparison)—Naked steel sheet with same treatment as F  
 J (comparison)—Naked steel sheet with no treatment

TABLE 8

| Formability    |                         |                      |                                        |
|----------------|-------------------------|----------------------|----------------------------------------|
|                | Conical cup value (mm.) | Erichsen value (mm.) | Removal-ability of treatment materials |
| Steel sheets:  |                         |                      | Surface condition                      |
| A              | 36.8                    | 12.2                 | Dry.                                   |
| B              | 36.7                    | 12.0                 | Dry.                                   |
| C              | 36.4                    | 12.4                 | Good                                   |
| D              | 36.8                    | 11.7                 | Dry.                                   |
| E              | 36.7                    | 11.5                 | Dry.                                   |
| F              | 37.9                    | 10.5                 | Wet.                                   |
| G <sup>1</sup> | 38.3                    | 10.4                 | Dry.                                   |
| H <sup>1</sup> | 37.5                    | 10.5                 | Good                                   |
| I <sup>1</sup> | 38.0                    | 10.0                 | do                                     |
| J <sup>1</sup> | 38.1                    | 10.0                 | Dry.                                   |

<sup>1</sup> Comparison..

Formability tests were done in similar way as in Example 3.

## EXAMPLE 10

A number of testpieces were taken from the steel sheet B and the conical cup tests were conducted continuously with the treated surface faced on the die side. As comparison, testpieces B' which were non-treated similar lead-tin alloy plated steel sheet were subjected to the conical cup test with spindle oil applied on the testpieces on the die side. Results are shown in FIG. 4, in which the ordinate shows an average value for every five testpieces in series from the beginning of the test.

On the other hand testpieces B were continuously subjected to Erichsen tests with the treated surface faced on the punch side. As comparison, similar lead-tin alloy plated steel sheets B' which were not surface treated were also tested with vaseline applied on the steel surface on the punch side. Results are shown in FIG. 5, in which the ordinate shows an average value for every five testpieces.

In all cases, the present steel sheets which were treated with palmitic acid showed far less variation in their measurements and did not affect the tools by repetition of tests, while in case of comparison steel sheets in which spindle oil or vaseline was used remarkable variations in the measurement were seen at the beginning, which clearly indicate the burning of metallic layer.

30

35

40

45

What is claimed is:

1. Surface treated steel sheet suitable for forming works which comprises metallic coating applied on a steel sheet surface, said metallic coating being composed of material selected from the group consisting of zinc, lead, zinc base alloy and lead base alloy, and a layer of higher carboxylic acid based material applied on the metallic coating, said higher carboxylic acid based material being solid at room temperatures.
- 5 10 15 20 25 30 35 40 45 50 55 60 65 70 75 80 85 90 95 100 105 110 115 120 125 130 135 140 145 150 155 160 165 170 175 180 185 190 195 200 205 210 215 220 225 230 235 240 245 250 255 260 265 270 275 280 285 290 295 300 305 310 315 320 325 330 335 340 345 350 355 360 365 370 375 380 385 390 395 400 405 410 415 420 425 430 435 440 445 450 455 460 465 470 475 480 485 490 495 500 505 510 515 520 525 530 535 540 545 550 555 560 565 570 575 580 585 590 595 600 605 610 615 620 625 630 635 640 645 650 655 660 665 670 675 680 685 690 695 700 705 710 715 720 725 730 735 740 745 750 755 760 765 770 775 780 785 790 795 800 805 810 815 820 825 830 835 840 845 850 855 860 865 870 875 880 885 890 895 900 905 910 915 920 925 930 935 940 945 950 955 960 965 970 975 980 985 990 995 1000 1005 1010 1015 1020 1025 1030 1035 1040 1045 1050 1055 1060 1065 1070 1075 1080 1085 1090 1095 1100 1105 1110 1115 1120 1125 1130 1135 1140 1145 1150 1155 1160 1165 1170 1175 1180 1185 1190 1195 1200 1205 1210 1215 1220 1225 1230 1235 1240 1245 1250 1255 1260 1265 1270 1275 1280 1285 1290 1295 1300 1305 1310 1315 1320 1325 1330 1335 1340 1345 1350 1355 1360 1365 1370 1375 1380 1385 1390 1395 1400 1405 1410 1415 1420 1425 1430 1435 1440 1445 1450 1455 1460 1465 1470 1475 1480 1485 1490 1495 1500 1505 1510 1515 1520 1525 1530 1535 1540 1545 1550 1555 1560 1565 1570 1575 1580 1585 1590 1595 1600 1605 1610 1615 1620 1625 1630 1635 1640 1645 1650 1655 1660 1665 1670 1675 1680 1685 1690 1695 1700 1705 1710 1715 1720 1725 1730 1735 1740 1745 1750 1755 1760 1765 1770 1775 1780 1785 1790 1795 1800 1805 1810 1815 1820 1825 1830 1835 1840 1845 1850 1855 1860 1865 1870 1875 1880 1885 1890 1895 1900 1905 1910 1915 1920 1925 1930 1935 1940 1945 1950 1955 1960 1965 1970 1975 1980 1985 1990 1995 2000 2005 2010 2015 2020 2025 2030 2035 2040 2045 2050 2055 2060 2065 2070 2075 2080 2085 2090 2095 2100 2105 2110 2115 2120 2125 2130 2135 2140 2145 2150 2155 2160 2165 2170 2175 2180 2185 2190 2195 2200 2205 2210 2215 2220 2225 2230 2235 2240 2245 2250 2255 2260 2265 2270 2275 2280 2285 2290 2295 2300 2305 2310 2315 2320 2325 2330 2335 2340 2345 2350 2355 2360 2365 2370 2375 2380 2385 2390 2395 2400 2405 2410 2415 2420 2425 2430 2435 2440 2445 2450 2455 2460 2465 2470 2475 2480 2485 2490 2495 2500 2505 2510 2515 2520 2525 2530 2535 2540 2545 2550 2555 2560 2565 2570 2575 2580 2585 2590 2595 2600 2605 2610 2615 2620 2625 2630 2635 2640 2645 2650 2655 2660 2665 2670 2675 2680 2685 2690 2695 2700 2705 2710 2715 2720 2725 2730 2735 2740 2745 2750 2755 2760 2765 2770 2775 2780 2785 2790 2795 2800 2805 2810 2815 2820 2825 2830 2835 2840 2845 2850 2855 2860 2865 2870 2875 2880 2885 2890 2895 2900 2905 2910 2915 2920 2925 2930 2935 2940 2945 2950 2955 2960 2965 2970 2975 2980 2985 2990 2995 3000 3005 3010 3015 3020 3025 3030 3035 3040 3045 3050 3055 3060 3065 3070 3075 3080 3085 3090 3095 3100 3105 3110 3115 3120 3125 3130 3135 3140 3145 3150 3155 3160 3165 3170 3175 3180 3185 3190 3195 3200 3205 3210 3215 3220 3225 3230 3235 3240 3245 3250 3255 3260 3265 3270 3275 3280 3285 3290 3295 3300 3305 3310 3315 3320 3325 3330 3335 3340 3345 3350 3355 3360 3365 3370 3375 3380 3385 3390 3395 3400 3405 3410 3415 3420 3425 3430 3435 3440 3445 3450 3455 3460 3465 3470 3475 3480 3485 3490 3495 3500 3505 3510 3515 3520 3525 3530 3535 3540 3545 3550 3555 3560 3565 3570 3575 3580 3585 3590 3595 3600 3605 3610 3615 3620 3625 3630 3635 3640 3645 3650 3655 3660 3665 3670 3675 3680 3685 3690 3695 3700 3705 3710 3715 3720 3725 3730 3735 3740 3745 3750 3755 3760 3765 3770 3775 3780 3785 3790 3795 3800 3805 3810 3815 3820 3825 3830 3835 3840 3845 3850 3855 3860 3865 3870 3875 3880 3885 3890 3895 3900 3905 3910 3915 3920 3925 3930 3935 3940 3945 3950 3955 3960 3965 3970 3975 3980 3985 3990 3995 4000 4005 4010 4015 4020 4025 4030 4035 4040 4045 4050 4055 4060 4065 4070 4075 4080 4085 4090 4095 4100 4105 4110 4115 4120 4125 4130 4135 4140 4145 4150 4155 4160 4165 4170 4175 4180 4185 4190 4195 4200 4205 4210 4215 4220 4225 4230 4235 4240 4245 4250 4255 4260 4265 4270 4275 4280 4285 4290 4295 4300 4305 4310 4315 4320 4325 4330 4335 4340 4345 4350 4355 4360 4365 4370 4375 4380 4385 4390 4395 4400 4405 4410 4415 4420 4425 4430 4435 4440 4445 4450 4455 4460 4465 4470 4475 4480 4485 4490 4495 4500 4505 4510 4515 4520 4525 4530 4535 4540 4545 4550 4555 4560 4565 4570 4575 4580 4585 4590 4595 4600 4605 4610 4615 4620 4625 4630 4635 4640 4645 4650 4655 4660 4665 4670 4675 4680 4685 4690 4695 4700 4705 4710 4715 4720 4725 4730 4735 4740 4745 4750 4755 4760 4765 4770 4775 4780 4785 4790 4795 4800 4805 4810 4815 4820 4825 4830 4835 4840 4845 4850 4855 4860 4865 4870 4875 4880 4885 4890 4895 4900 4905 4910 4915 4920 4925 4930 4935 4940 4945 4950 4955 4960 4965 4970 4975 4980 4985 4990 4995 5000 5005 5010 5015 5020 5025 5030 5035 5040 5045 5050 5055 5060 5065 5070 5075 5080 5085 5090 5095 5100 5105 5110 5115 5120 5125 5130 5135 5140 5145 5150 5155 5160 5165 5170 5175 5180 5185 5190 5195 5200 5205 5210 5215 5220 5225 5230 5235 5240 5245 5250 5255 5260 5265 5270 5275 5280 5285 5290 5295 5300 5305 5310 5315 5320 5325 5330 5335 5340 5345 5350 5355 5360 5365 5370 5375 5380 5385 5390 5395 5400 5405 5410 5415 5420 5425 5430 5435 5440 5445 5450 5455 5460 5465 5470 5475 5480 5485 5490 5495 5500 5505 5510 5515 5520 5525 5530 5535 5540 5545 5550 5555 5560 5565 5570 5575 5580 5585 5590 5595 5600 5605 5610 5615 5620 5625 5630 5635 5640 5645 5650 5655 5660 5665 5670 5675 5680 5685 5690 5695 5700 5705 5710 5715 5720 5725 5730 5735 5740 5745 5750 5755 5760 5765 5770 5775 5780 5785 5790 5795 5800 5805 5810 5815 5820 5825 5830 5835 5840 5845 5850 5855 5860 5865 5870 5875 5880 5885 5890 5895 5900 5905 5910 5915 5920 5925 5930 5935 5940 5945 5950 5955 5960 5965 5970 5975 5980 5985 5990 5995 6000 6005 6010 6015 6020 6025 6030 6035 6040 6045 6050 6055 6060 6065 6070 6075 6080 6085 6090 6095 6100 6105 6110 6115 6120 6125 6130 6135 6140 6145 6150 6155 6160 6165 6170 6175 6180 6185 6190 6195 6200 6205 6210 6215 6220 6225 6230 6235 6240 6245 6250 6255 6260 6265 6270 6275 6280 6285 6290 6295 6300 6305 6310 6315 6320 6325 6330 6335 6340 6345 6350 6355 6360 6365 6370 6375 6380 6385 6390 6395 6400 6405 6410 6415 6420 6425 6430 6435 6440 6445 6450 6455 6460 6465 6470 6475 6480 6485 6490 6495 6500 6505 6510 6515 6520 6525 6530 6535 6540 6545 6550 6555 6560 6565 6570 6575 6580 6585 6590 6595 6600 6605 6610 6615 6620 6625 6630 6635 6640 6645 6650 6655 6660 6665 6670 6675 6680 6685 6690 6695 6700 6705 6710 6715 6720 6725 6730 6735 6740 6745 6750 6755 6760 6765 6770 6775 6780 6785 6790 6795 6800 6805 6810 6815 6820 6825 6830 6835 6840 6845 6850 6855 6860 6865 6870 6875 6880 6885 6890 6895 6900 6905 6910 6915 6920 6925 6930 6935 6940 6945 6950 6955 6960 6965 6970 6975 6980 6985 6990 6995 7000 7005 7010 7015 7020 7025 7030 7035 7040 7045 7050 7055 7060 7065 7070 7075 7080 7085 7090 7095 7100 7105 7110 7115 7120 7125 7130 7135 7140 7145 7150 7155 7160 7165 7170 7175 7180 7185 7190 7195 7200 7205 7210 7215 7220 7225 7230 7235 7240 7245 7250 7255 7260 7265 7270 7275 7280 7285 7290 7295 7300 7305 7310 7315 7320 7325 7330 7335 7340 7345 7350 7355 7360 7365 7370 7375 7380 7385 7390 7395 7400 7405 7410 7415 7420 7425 7430 7435 7440 7445 7450 7455 7460 7465 7470 7475 7480 7485 7490 7495 7500 7505 7510 7515 7520 7525 7530 7535 7540 7545 7550 7555 7560 7565 7570 7575 7580 7585 7590 7595 7600 7605 7610 7615 7620 7625 7630 7635 7640 7645 7650 7655 7660 7665 7670 7675 7680 7685 7690 7695 7700 7705 7710 7715 7720 7725 7730 7735 7740 7745 7750 7755 7760 7765 7770 7775 7780 7785 7790 7795 7800 7805 7810 7815 7820 7825 7830 7835 7840 7845 7850 7855 7860 7865 7870 7875 7880 7885 7890 7895 7900 7905 7910 7915 7920 7925 7930 7935 7940 7945 7950 7955 7960 7965 7970 7975 7980 7985 7990 7995 8000 8005 8010 8015 8020 8025 8030 8035 8040 8045 8050 8055 8060 8065 8070 8075 8080 8085 8090 8095 8100 8105 8110 8115 8120 8125 8130 8135 8140 8145 8150 8155 8160 8165 8170 8175 8180 8185 8190 8195 8200 8205 8210 8215 8220 8225 8230 8235 8240 8245 8250 8255 8260 8265 8270 8275 8280 8285 8290 8295 8300 8305 8310 8315 8320 8325 8330 8335 8340 8345 8350 8355 8360 8365 8370 8375 8380 8385 8390 8395 8400 8405 8410 8415 8420 8425 8430 8435 8440 8445 8450 8455 8460 8465 8470 8475 8480 8485 8490 8495 8500 8505 8510 8515 8520 8525 8530 8535 8540 8545 8550 8555 8560 8565 8570 8575 8580 8585 8590 8595 8600 8605 8610 8615 8620 8625 8630 8635 8640 8645 8650 8655 8660 8665 8670 8675 8680 8685 8690 8695 8700 8705 8710 8715 8720 8725 8730 8735 8740 8745 8750 8755 8760 8765 8770 8775 8780 8785 8790 8795 8800 8805 8810 8815 8820 8825 8830 8835 8840 8845 8850 8855 8860 8865 8870 8875 8880 8885 8890 8895 8900 8905 8910 8915 8920 8925 8930 8935 8940 8945 8950 8955 8960 8965 8970 8975 8980 8985 8990 8995 9000 9005 9010 9015 9020 9025 9030 9035 9040 9045 9050 9055 9060 9065 9070 9075 9080 9085 9090 9095 9100 9105 9110 9115 9120 9125 9130 9135 9140 9145 9150 9155 9160 9165 9170 9175 9180 9185 9190 9195 9200 9205 9210 9215 9220 9225 9230 9235 9240 9245 9250 9255 9260 9265 9270 9275 9280 9285 9290 9295 9300 9305 9310 9315 9320 9325 9330 9335 9340 9345 9350 9355 9360 9365 9370 9375 9380 9385 9390 9395 9400 9405 9410 9415 9420 9425 9430 9435 9440 9445 9450 9455 9460 9465 9470 9475 9480 9485 9490 9495 9500 9505 9510 9515 9520 9525 9530 9535 9540 9545 9550 9555 9560 9565 9570 9575 9580 9585 9590 9595 9600 9605 9610 9615 9620 9625 9630 9635 9640 9645 9650 9655 9660 9665 9670 9675 9680 9685 9690 9695 9700 9705 9710 9715 9720 9725 9730 9735 9740 9745 9750 9755 9760 9765 9770 9775 9780 9785 9790 9795 9800 9805 9810 9815 9820 9825 9830 9835 9840 9845 9850 9855 9860 9865 9870 9875 9880 9885 9890 9895 9900 9905 9910 9915 9920 9925 9930 9935 9940 9945 9950 9955 9960 9965 9970 9975 9980